

## 1

3,109,757

**METHOD AND MATERIAL FOR APPLYING PHOSPHATE CONVERSION COATINGS ON ZINCIFEROUS SURFACES**

Earl R. Reinhold, Levittown, Pa., assignor to Amchem Products, Inc., Ambler, Pa., a corporation of Delaware  
No Drawings. Filed Jan. 26, 1962, Ser. No. 169,997

6 Claims. (Cl. 148—6.15)

This invention relates to the art of coating zinciferous surfaces and involves a method and solutions for producing phosphate conversion coatings on such surfaces which coatings have highly improved characteristics, especially with respect to fineness of grain structure without serious sacrifice of coating weight, ability to promote the adhesion of siccative finishes and resistance to stresses set up by bending, folding or shaping the metal after the coating has been applied.

As used herein the expression "zinciferous surfaces" or "zinc surfaces" are to be understood as applying to alloys of zinc with other metals wherein zinc is the principal ingredient, to hot-dipped galvanized surfaces, to electro-deposited zinc surfaces, as well as to essentially pure zinc surfaces.

The art of applying phosphate conversion coatings to zinc surfaces, of course, is well developed and is based upon the familiar practice of subjecting the surfaces to the action of an aqueous acid phosphate coating solution until the desired coating has been deposited. Following this the surface is customarily rinsed either with water or with dilute chromic and/or phosphoric acid rinses. Probably the most familiar of the aqueous acid phosphate coating solutions is a zinc solution and the present invention is directed to the improvement of methods involving such a solution.

In this art of coating zinc surfaces with aqueous acid zinc phosphate coating solutions various solution formulations are well known to the art and the present invention is broadly applicable to solutions of this general type although, as will be pointed out below, maximum benefits from the present invention are obtainable where the aqueous acid zinc phosphate solutions conform to the specifications recited hereinafter.

In the phosphate coating of zinc surfaces the art has long realized that the conversion coated surfaces and any siccative finish that may have been applied thereto do not lend themselves very well to bending or folding without serious attendant cracking and peeling with subsequent loss of or injury to the siccative film. This is particularly exemplified by what happens to an acrylic base paint which is often objectionably impaired as the result of cracking of the phosphate coating in situations requiring bending or shaping operations such, for example, as in the use of galvanized iron sheeting as siding in the construction industry.

With the foregoing in mind, the principal object of the present invention is the provision of a method and solutions for applying an improved, adhesion-promoting, zinc phosphate conversion coating on zinc surfaces which will withstand or resist to a marked extent flexing, shaping and bending operations even to an extent involving a 180° bend without failure of the siccative finish or film.

The invention is broadly based upon the discovery that if the following agents are added to an aqueous acid zinc phosphate coating solution of generally standard characteristics and such solution is then utilized in the treatment of zinciferous surfaces it will form on the surfaces zinc phosphate conversion coatings which are smoother, finer grained, more tightly adherent, unimpaired as to coating weight, and better suited to serve as a substrate for subsequent siccative finishes than are the familiar zinc

## 2

phosphate conversion coatings presently known to the art. The addition agents employed with my invention are:

(a) From 0.1% to 1.0% by weight of a compound selected from the group consisting of glycerophosphoric acids and water-soluble salts thereof; and

(b) At least 0.025% by weight of complex fluoride radical selected from the group consisting of fluoroboric, fluosilicic, fluotitanic and fluozirconic acids and alkali metal and ammonium salts thereof.

The glycerophosphoric acids or water-soluble salts thereof include mono and di-glycerophosphate compounds. Soluble salts are preferred over the acids in view of their greater solubility in the acid phosphate coating media. Particularly preferred salts include the alkali metal and ammonium mono and di-glycerophosphates, since these are more readily prepared, and provide an easily handled concentrated liquid solution.

Where the amount of glycerophosphate, or water-soluble salt thereof, which is employed, is less than the 0.1% by weight, minimum concentration, the improved paint-adhesion promoting coatings will not be obtained, and subsequent bending or flexing of the phosphate coated and painted zinc surfaces will result in cracking and peeling of the siccative film. As the amount of glycerophosphate compound in the phosphate coating solution is increased, the paint bonding qualities of subsequently produced coatings on zinc surfaces also increases up to an apparent maximum improvement at about 1% concentration, by weight. Use of glycerophosphates in amounts greater than 1% concentration has no noticeable deleterious effect upon either the coating reaction, or upon subsequent paint adhesion on the coated surfaces. However, as no additional benefit is obtained when employing more than about 1% glycerophosphate, it is preferred, in the interests of economy and to prevent waste, to operate between a range of from 0.1% to 1.0% concentration thereof as stated above.

As for the quantity of complex fluorides, I have found that, in order to realize the benefits of this invention, they should be added in an amount equal to at least 0.25% by weight of the coating solution. If less than this minimum quantity is present the resulting conversion coatings will not provide the highly flexible, paint-bonding qualities obtainable by my invention.

Insofar as an upper concentration limit of complex fluoride is concerned, I have found that there is nothing critical about the quantity employed since solubility considerations pretty well limit the amounts thereof which can be dissolved in zinc phosphate coating solutions of this general character. For example, the complex fluoride acids, i.e. fluoroboric, fluosilicic, etc., and the ammonium salts thereof have been found to be more soluble in the coating baths or solutions than the alkali metal salts. However, the maximum solubility of any of these complex fluoride compounds in the customary aqueous acid zinc phosphate coating solutions is about 2.5% by weight thereof. Use of a relatively low concentration of complex fluoride compound, for instance, about 0.03%, provides the same enhanced adhesion-promoting characteristics as does the use of large amounts, even those amounts which approach the saturation limitation. Therefore, in the interests of preventing waste and securing maximum economy of operation, I prefer to employ a range of complex fluoride concentration of from 0.025% to 0.25% by weight of the coating solution.

While the use of complex fluorides from the class described is essential for successful operation of the process of this invention, it has been found that the inclusion of simple fluoride ions into the coating solution of this invention has no apparent deleterious effect upon coating formation. However, use of simple fluoride ion alone

## 3

will not provide the improved results obtainable with the complex fluorides as defined hereinabove.

As a further guide in attainment of the maximum benefits of my invention I wish to call attention to the following facts.

The phosphate ion content which yields the best results ranges from about 0.5% to about 2.5% by weight of the coating solution with the minimum quantity being at least sufficient to form the dihydrogen phosphate with the zinc ions present and the content of zinc ions should be in an amount which does not exceed about 0.5% by weight of the coating solution.

Another factor which should be observed in obtaining the maximum benefits of my invention arises in connection with the presence of any oxidizing ion such as nitrate and mixtures of nitrate and nitrite. These oxidizing agents, of course, are very familiar to those skilled in the art and for best results with my invention the quantity of nitrate ion should be about 0.2% to about 1.0% with major benefits being obtainable where the quantity lies between about 0.3% to about 0.5%. Where nitrite is also included in the bath as an oxidizing agent substantially smaller amounts thereof are required in order to yield the results which are secured by this familiar ingredient. For example, the range of nitrite ion when used in combination with nitrate ion is from about 0.0002% to about 0.008% and with my invention I have found that optimum flexible paint-bonding properties in the phosphate conversion coatings are obtainable with the use of less than about 0.5% nitrate ion and less than about 0.005% of nitrite ion.

Insofar as total acidity of the solution is concerned, I have found that it is preferable to utilize zinc phosphate coating solutions which have a total acidity of less than 40 points. Total acidity is the milliliters of tenth normal sodium hydroxide (points) required to titrate a 10 ml. sample of the bath to a phenolphthalein endpoint, whereas the free acidity is the mls. of tenth normal sodium hydroxide (points) required to neutralize a 10 ml. sample of the bath to a brom cresol green endpoint.

Beyond the foregoing, if an aqueous acid zinc phosphate coating solution is employed which contains nickel and/or copper ion (these ions of course being well known to the art), it is important to observe the following facts in order to secure the maximum benefits of my invention. In the case of nickel ion there should be employed somewhere between about 0.01% and 0.4% and in the case of copper between about 0.0003% and 0.005%. Use of higher amounts than these of nickel and copper will not yield the full advantages otherwise obtainable with the process and solutions of my invention. Actually, best results are secured with the utilization (where these

## 4

metals are employed) of less than 0.3% of nickel and as little as 0.0003% to 0.001% of copper.

A concentrate which is suitable for dilution with water, as hereinafter described, to produce the coating solutions of this invention, and which is also suitable for addition to partially exhaust solutions as a replenisher, can be prepared according to the following example:

## EXAMPLE I

|    |                                                      | Percent by weight |
|----|------------------------------------------------------|-------------------|
| 10 | ZnO                                                  | 8.0               |
|    | H <sub>3</sub> PO <sub>4</sub> (75%)                 | 39.5              |
| 5  | Ni(NO <sub>3</sub> ) <sub>2</sub> ·6H <sub>2</sub> O | 6.75              |
|    | HNO <sub>3</sub> (38° Bé.)                           | 2.87              |
| 15 | Water                                                | 42.88             |
|    |                                                      | 100.00            |

The above formula, when diluted with water to a strength of 4% by volume and having added thereto 0.25% (weight/volume) of caustic soda, has the following analysis:

|                |       |
|----------------|-------|
| Total acidity  | 25    |
| Free acidity   | 3.0   |
| Percent nickel | 0.075 |

The acidity referred to was determined by the method indicated above.

To a dilute solution prepared as above described there should then be added from 0.1% to 1.0% by weight of 30 a glycerophosphate compound as hereinabove described and at least 0.025% by weight of a complex fluoride as previously described. The solution should then be heated to between about 120° F. and 160° F. and preferably between 130° F. and 160° F. and can then be utilized with 35 greatest benefit in applying zinc phosphate conversion coatings to zinciferous surfaces and it will be found that it will produce excellent, highly flexible, smooth and fine-grained, paint-bonding phosphate conversion coatings which are ideally suitable as a substrate for siccative 40 finishes.

The advantages attainable with my invention are amply demonstrated by the following comparative tests which I have conducted. A 4% dilution of the concentrate of Example I given above was prepared and aliquot samples 45 of the diluted solution were utilized in accordance with the examples given in Table I below. The metal being coated was hot-dipped galvanized steel. A series of similar panels from such galvanized steel were prepared and cleaned in accordance with well established prior art practices. 50 The reported paint adhesion results were determined following application of an epoxy primary paint system.

Table I

| Example No. | Percent glycerophosphate | Complex fluoride |                                                  | Coating wt., mg./ft. <sup>2</sup> | Paint adhesion test (ASTM D-522-41) |                     |
|-------------|--------------------------|------------------|--------------------------------------------------|-----------------------------------|-------------------------------------|---------------------|
|             |                          | Percent          | Type                                             |                                   | Percent paint loss                  | Paint appearance    |
| 2           | None                     | None             | (NH <sub>4</sub> ) <sub>2</sub> ZnF <sub>6</sub> | 462                               | 50                                  | Heavy cracking.     |
| 3           | None                     | 0.05             | (NH <sub>4</sub> ) <sub>2</sub> ZnF <sub>6</sub> | 487                               | 10                                  | Moderate cracking.  |
| 4           | None                     | 0.126            | H <sub>2</sub> SiF <sub>6</sub>                  | 469                               | 30                                  | Heavy cracking.     |
| 5           | None                     | 0.033            | H <sub>2</sub> TiF <sub>6</sub>                  | 442                               | 20                                  | Do.                 |
| 6           | 0.1                      | None             | (NH <sub>4</sub> ) <sub>2</sub> ZnF <sub>6</sub> | 501                               | 5                                   | Fine cracking.      |
| 7           | 0.1                      | 0.05             | (NH <sub>4</sub> ) <sub>2</sub> ZnF <sub>6</sub> | 501                               | 1                                   | Very fine cracking. |
| 8           | 0.2                      | 0.05             | (NH <sub>4</sub> ) <sub>2</sub> ZnF <sub>6</sub> | 420                               | <1                                  | Do.                 |
| 9           | 0.4                      | 0.05             | (NH <sub>4</sub> ) <sub>2</sub> ZnF <sub>6</sub> | 402                               | 1                                   | Do.                 |
| 10          | 0.1                      | 0.126            | H <sub>2</sub> SiF <sub>6</sub>                  | 477                               | 2                                   | Fine cracking.      |
| 11          | 0.2                      | 0.126            | H <sub>2</sub> SiF <sub>6</sub>                  | 456                               | <1                                  | Very fine cracking. |
| 12          | 0.4                      | 0.126            | H <sub>2</sub> SiF <sub>6</sub>                  | 468                               | 1                                   | Do.                 |
| 13          | 0.2                      | 0.025            | H <sub>2</sub> B <sub>2</sub> F <sub>9</sub>     | 417                               | (2)                                 | Very fine cracking. |
| 14          | 0.2                      | 0.033            | H <sub>2</sub> TiF <sub>6</sub>                  | 494                               | <1                                  | Do.                 |
| 15          | 0.2                      | 0.33             | H <sub>2</sub> TiF <sub>6</sub>                  | 438                               | <1                                  | Very fine cracking. |
| 16          | 0.4                      | 0.33             | H <sub>2</sub> TiF <sub>6</sub>                  | 501                               | <1                                  | Do.                 |

<sup>1</sup> Examples 8 and 14 also contained 0.005% copper ion.

<sup>2</sup> The panels of Example 13 were inadvertently lost and were not available for this test but visual observation thereof indicated that their coatings would be equally satisfactory as those in Examples 7 to 16, inclusive.

The glycerophosphate utilized in the above examples was the disodium salt. However, equally satisfactory results are obtained when utilizing the monosodium salt, the acid or other alkali metal or ammonium salts.

As can be seen from the data reported above, when the glycerophosphate compound and the complex fluoride were added to the coating solution there was substantially no loss of coating weight, nor was there any loss during the paint adhesion test. This discovery was somewhat surprising in view of the well known fact that other coating refining agents such, for example, as the polyphosphates, when added to phosphate coating solutions, have a tendency to reduce the coating weight and even, in some cases, to completely poison the coating bath.

All of the results reported in Table I above were obtained utilizing constant bath temperatures of 63° C. (145° F.) and a spray time of 30 seconds. However, the treating time may vary between about 7 seconds to about 10 minutes, and the concentrated solution may be diluted to a strength of about 1/2% to about 6% volume with water. The preferred treating time is from about 10 seconds to about 2 minutes, and the preferred dilution is from about 1% to about 4% by volume.

Application of the solutions of this invention to zinc surfaces may be by dip, spray, or any other manner, so long as the zinc surface to be coated is thoroughly wetted by the coating solution.

After the treatment, the surface should be rinsed with water or with one of the final rinses which are customary in the art. Examples of such rinses are dilute solutions of chromic acid and/or phosphoric acid.

The concentrate of Example I (or a similar one containing copper in addition) when employed as a replenishing material for partially depleted solutions restores not only the desired level of the coating producing ingredients, but also the accelerators such as nickel and copper.

In the solutions of this invention the nickel and copper ions can be provided by adding a salt which is soluble in the solution, for example, a carbonate, nitrate, chloride or sulfate.

While the surfaces to be treated according to this invention should be clean, the cleaning procedure is not a part of this invention, and it will suffice to state that any of the well known and commercially available cleaning solutions for zinc surfaces may be employed.

I claim:

1. In the art of phosphate coating zinciferous surfaces, the method which comprises subjecting said surface to the action of an aqueous acid zinc phosphate coating solution, the coating producing ingredients of which consist essentially of phosphate ion from 0.5% to 2.5% by weight

and nitrate ion from 0.2% to 1.0% by weight, which solution also contains as addition agents:

(a) at least 0.1% by weight of the solution of a compound selected from the group which consists of glycerophosphoric acids and water soluble salts thereof; and

(b) at least 0.025% by weight of the solution of complex fluoride radical selected from the group consisting of fluoroboric, fluosilicic, fluotitanic and fluozirconic acids and alkali metal and ammonium salts thereof;

and replenishing the solution as required to maintain its ingredients as defined.

2. The method of claim 1 wherein the content of agent (a) is maintained at from 0.1% to 1.0% and that of agent (b) from 0.025% to 0.25%.

3. The method of claim 1 wherein the total acidity of the solution is less than 40 points as measured by the quantity of tenth normal sodium hydroxide required to titrate a 10 ml. sample of the solution of a phenolphthalein endpoint.

4. An aqueous acid zinc phosphate coating solution, the coating producing ingredients consisting essentially of phosphate ion from 0.5% to 2.5% by weight and nitrate ion from 0.2% to 1.0% by weight, which solution also contains as addition agents:

(a) at least 0.1% by weight of the solution of a compound selected from the group which consists of glycerophosphoric acids and water soluble salts thereof; and

(b) at least 0.025% by weight of the solution of complex fluoride radical selected from the group consisting of fluoroboric, fluosilicic, fluotitanic and fluozirconic acids and alkali metal and ammonium salts thereof.

5. A solution according to claim 4 which, further, contains from 0.01% to 0.4% of nickel ion.

6. A solution according to claim 4 which, further, contains from 0.0003% to 0.005% of copper ion.

#### References Cited in the file of this patent

##### UNITED STATES PATENTS

|           |                      |              |
|-----------|----------------------|--------------|
| 1,221,046 | Gravell -----        | Apr. 3, 1917 |
| 1,329,573 | Allen -----          | Feb. 3, 1920 |
| 2,798,016 | Lesser -----         | July 2, 1957 |
| 2,798,830 | Newhard et al. ----- | July 9, 1957 |
| 2,863,793 | De Cerma -----       | Dec. 9, 1958 |

##### FOREIGN PATENTS

|         |                     |              |
|---------|---------------------|--------------|
| 586,832 | Great Britain ----- | Apr. 2, 1947 |
|---------|---------------------|--------------|

UNITED STATES PATENT OFFICE  
CERTIFICATE OF CORRECTION

Patent No. 3,109,757

November 5, 1963

Earl R. Reinhold

It is hereby certified that error appears in the above numbered patent requiring correction and that the said Letters Patent should read as corrected below.

Column 2, line 40, for "0.25%" read -- 0.025% --; column 4, line 6, for "exhaust" read -- exhausted --.

Signed and sealed this 28th day of April 1964.

(SEAL)

Attest:

ERNEST W. SWIDER

Attesting Officer

EDWARD J. BRENNER  
Commissioner of Patents